

Dec. 11, 1928.

1,695,044

K. HALLMANN  
PROCESS FOR INCREASING THE ELECTRICAL CONDUCTIVITY  
AND THE FLEXIBILITY OF METALS OR ALLOYS  
Filed Sept. 21, 1922



Karl Hallmann

Inventor

by his attorney.

Mark B. Bley

## UNITED STATES PATENT OFFICE.

KARL HALLMANN, OF MUNICH, GERMANY.

PROCESS FOR INCREASING THE ELECTRICAL CONDUCTIVITY AND THE FLEXIBILITY  
OF METALS OR ALLOYS.

Application filed September 21, 1922, Serial No. 589,702, and in Germany August 11, 1922.

The present invention refers to a process for improving the electrical conductivity and the flexibility of metals or alloys which have been cast in the fluid state and after 5 having been solidified have been subjected to a heat treatment. It is known that to increase the hardness, the tenacity of metals or alloys and the possibility of working them with cutting tools, it is necessary to reheat 10 the metals or alloys after casting or annealing and quenching to relatively low temperatures which are below the known annealing temperatures. The metals or alloys, which have been thus treated, do however not show 15 such a flexibility and electrical conductivity as is required for certain electrotechnical purposes, as for instance for electrical conducting wires in free air. The said disadvantages are overcome by the present process.

20 The process consists in that the heated metals as they come from the casting or annealing process, are cooled down to ordinary temperatures or near to them (for instance about 50 degrees centigrade) and then subjected to a treatment which causes a reduction 25 of their diameter, after which the metals or alloys are subjected to heat at temperatures below those at which by the action of heat the strength and temper of the metals 30 or alloys is diminished. The effect of the present process may be illustrated by the following figures: A wire of pure aluminum for electrical free air conductors has an electrical conductivity of 33-34 at 20 degrees centigrade 35 and may bear 5-7 bendings over a radius equal to the diameter of the wire before a breakage will occur. The wires of aluminum with 0.5-1% silicon, 0.2-10% iron and 0.1-0.7% magnesium after having been 40 hardened by heating, cooling and heating again to relatively low temperatures, have an electrical conductivity of 28-29 and a flexibility of 0.5-1. If however, the last mentioned wire is subjected to the present process, 45 the electrical conductivity is increased to 32-33, nearly equal to that of pure aluminum wire whereas the flexibility is 3-4. The strength of the wire subjected to the present process is not injured.

50 The reduction of the diameter of the metals or alloys in rods, bars or blocks may be effected by a drawing or rolling process. For electrical conducting wires intended for use in free air a reduction of the diameter of 55 about 90% has been found as suitable.

The metals which come from the annealing process or casting are preferably not reduced in diameter immediately after having been cooled to about ordinary temperatures, but after having been allowed to age some time, 60 for instance from 2 to 3 days. (The last named aging treatment may be omitted, so that the cooled wires may be subjected immediately to a diminution of their diameter.) After this, the metals are heated to a temperature 65 of about 160 to 200 degrees centigrade. The decrease of the temperature from the annealing process or casting, may be effected by chilling for instance with oil or water or by the action of air. The agents for lowering the temperature are selected according to the size of the objects. For example water is used for small objects and oil is used for large objects. The cooling must be effected 70 so quickly that the hot metal which has been subjected to the casting or annealing temperature, should not remain above a temperature of 200° C. for a period sufficiently long to lessen the effect secured by subsequent treatment at 160°-200° C.

75 The order of the several steps is important for the success of my process. First, the metals or alloys must be brought to the high annealing temperature of the annealing process or casting, then to a temperature at which no alteration of the internal structure will 80 be effected, then subjected to the reduction of their diameter at low temperature (at ordinary temperature or so called in the cold) and finally subjected to a heating to temperatures between 160 and 200 degrees centigrade.

85 In the following, some methods of carry out the present process are explained for an alloy of aluminum with 0.5 to 1% silicon, 0.2-0.0% iron, 0.1-0.7% magnesium. The 90 metals can as usual after the first annealing be drawn or pressed, which treatments cause also a diminution of their diameter and they are then subjected to the several steps of the present process.

95 1. The bars coming from the rolling process are rolled at about 540-560 degrees centigrade to wire of about 10-20 millimeters diameter then quickly cooled to ordinary temperature or at least to about 160-200 degrees centigrade in which latter case the wire is 100 allowed to cool further in the air. After a lapse of about 2 to 3 days the cold wire is rolled to 5 or 6 millimeters diameter and it is then drawn to the desired final diameter 105 110

or drawn directly from 10 or 20 millimeters to the final diameter. The completed wire is then subjected for about 8-12 hours to a temperature of 160 to 200 degrees centigrade and finally cooled.

2. The rolled bars are rolled at the usual rolling temperatures, say at about 350 to 450 degrees centigrade to round wire of about 10-20 millimeters diameter, cooled or allowed to cool and then annealed for about 2-3 hours at 540 to 560 degrees centigrade. After having been cooled quickly to about 160-200 degrees centigrade or about 20 degrees centigrade the wire of about 10-20 millimeters diameter is allowed to rest for about 2-3 days and then rolled in the cold until the final diameter is obtained whereupon it is subjected for about 8-12 hours to 160 to 200 degrees centigrade and cooled.
3. The bars are annealed to about 550 to 580 degrees centigrade and pressed at temperatures of about 540 to 560 degrees centigrade to round wire of about 10 to 20 millimeters diameter, the wire being forced either directly into water or oil or it is pressed in the atmosphere and quickly cooled after the pressing operation by bringing it into water or oil, to temperatures of at least 160 to 200 degrees centigrade. After about 2 or 3 days the wire is drawn in the cold to the desired final diameter and subjected for about 8-12 hours to 160 to 200 degrees centigrade and cooled.

4. The bars are pressed as described in connection with Example 3 and slowly or quickly cooled. The pressed wire of about 10 to 20 millimeters diameters is annealed for about 2 to 3 hours at 540 to 560 degrees centigrade and quickly cooled in water or oil or another suitable liquid to at least 160 to 200 degrees centigrade. After a lapse of about 2 to 3 days the wire is drawn or rolled in the cold to the desired final diameter and it is then subjected for about 8 to 12 hours to temperatures of about 160 to 200 degrees centigrade and finally cooled.

The diameter of the preliminarily rolled or pressed wire is so chosen that it receives by the rolling or drawing in the cold a diminution of its diameter of about 90% at least when compared with the original preliminarily rolled or pressed wire.

For an aluminum alloy composed of 96-91.3% aluminum, 0.5 to 1% silicon, 0.2 to 1% iron, 0.1 to 0.7% magnesium, 1-6% copper the first annealing temperature which is suitable is about 500 to 520 degrees centigrade. The further treatment is the same as described under Examples 1-4. If the pre-

liminarily rolled or pressed wire is annealed for a second time as described in connection with Examples 2-4 a preliminary rolling or pressing, temperature of about 450 to 500 degrees centigrade is used.

In similar manner the process may be used for other metals or alloys suitable for being hardened, as for instance aluminum zinc, aluminum copper, aluminum silicon, aluminum cadmium, aluminum glucinum.

The annealing temperature used according to the present invention is practically identical with the so-called condition diagram of the alloy to be treated, the abscissas being formed by the percentage of the alloying metal, the ordinate being formed by the temperature in degrees centigrade. The object of the treatment is to obtain an increase of the hardness and at the same time of the electrical conductivity, whereas hitherto according to the known process especially of Van Oordt U. S. Patent 1,326,775 only an increase of the hardness and at the same time a diminution of the electrical conductivity could be obtained. The drawing shows a diagram illustrating the effect of the present process on a wire of 2-3 mm. diameter 1 corresponding to the strength of 30 kg./mm.<sup>2</sup> and 28 electrical conductivity obtained according to the process of Van Oordt U. S. A. Patent 1,326,775, 2 after the drawing at the cold or ordinary temperature and 3 after the hardening at temperatures between 160-200 degrees centigrade. The drawing shows that by the step of this invention the conductivity is increased without diminishing the hardness thereof. That is, the aluminum or the like has been first recrystallized, then drawn, and it has then been subjected to a secondary heat treatment for lessening the internal strains therein.

I claim:

1. The process for increasing the electrical conductivity and flexibility of aluminum alloys which consists in annealing aluminum alloys to recrystallization temperatures, reducing their cross-section by treatment in the cold and heating them to temperatures between 160 and 200 degrees centigrade.

2. The process for increasing the electrical conductivity of aluminum alloys by annealing said alloys to recrystallization temperatures, reducing the cross section of such metals by treatment in the cold and heating to temperatures below 200 degrees centigrade.

In testimony whereof I hereunto affix my signature.

DR. ING. KARL HALLMANN.